

## UNITED STATES PATENT OFFICE

ARTHUR N. PARRETT, OF WILMINGTON, DELAWARE, ASSIGNOR TO E. I. DU PONT DE NEMOURS & COMPANY, OF WILMINGTON, DELAWARE, A CORPORATION OF DELAWARE

## COATED FABRIC AND METHOD OF PREPARING SAME

No Drawing.

Application filed September 9, 1927. Serial No. 218,577.

The invention relates to a fabric coating composition and a method of preparing the same, and more particularly to a fabric coating composition utilized in the production of 5 artificial leathers suitable for automobile tops, automobile trimmings, upholstery, luggage and the like.

Heretofore various materials have been suggested and used for automobile tops, as 10 for example, oil coated fabrics, rubberized fabrics and pyroxylin coated fabrics. Fabrics coated with compositions containing small amounts of bituminous material have also been used to some extent. None of 15 these prior products have been found satisfactory, however, as each presents some serious drawback. Oil coated fabrics, for instance, have the disadvantage of being high in cost and very liable to cold crack. The 20 rubberized fabrics have been found to be poor bases for the varnish top coat with which it is customary to finish automobile tops. This is probably due to the difference in the elasticity of the rubber and the varnish. Pyroxylin 25 coated fabrics have the drawback of requiring a number of coatings to give the required thickness, each coat having to be dried separately. Bituminous coated fabrics containing more than small amounts of the 30 bituminous material have heretofore been avoided because such compositions were found to give a stiff, brittle product subject to cold cracking.

An object of the present invention is to 35 provide a fabric coating composition, which contains a large percentage of bituminous material, and which is free from the objections of the prior art.

Another object of the invention is to produce 40 an artificial leather which is flexible and has a calendered surface capable of serving as a satisfactory base for the varnish top coat.

These objects are attained by my invention, 45 which produces an artificial leather suitable for the purposes named, by applying to a flexible fabric backing a calender coating composition containing bituminous material as its principal ingredient, and baking the 50 coated fabric at a temperature above 100° C.

and below the decomposition point of the ingredients. In some instances a further step is introduced, which consists in applying a top varnish coat to the calender coat before baking. An important feature of the 55 present invention is the novel composition of the calender coat, which contains, in addition to the bituminous material, various modifying agents which will be more fully described and specified hereinafter.

In carrying out the present invention, the materials making up the bituminous calender coat are mixed or combined in a rubber mill or mixing machine in a similar manner to that ordinarily used in mixing rubber compositions. After mixing, the composition is calendered out on the particular base to be used. Subsequently, the calender coated material may be embossed, if desired, and thereafter varnished, after which it is baked 70 at a temperature sufficient to soften and season the bituminous material and to bring about vulcanization in those cases wherein the composition contains vulcanizable products. For the baking operation the goods 75 are ordinarily festooned in a chamber provided with heat such as a vulcanizing chamber.

More in detail, the present invention contemplates forming the calender coat principally of one or more bituminous materials such as stearin pitch, asphalt, petroleum flux and the like, the bituminous content of the calender coat ranging from thirty to eighty 80 per cent of the composition. In order to modify the properties of the bituminous material, various agents, such as an indurator, a softener and a filler may be employed.

The purpose of the indurating agent is to 85 harden and toughen the composition. For this action, organic vulcanized materials, such as vulcanized rubber, or a vulcanized oil, for instance factis, may be used. Vulcanizable products, such as rubber, vegetable oil, 90 drying oil, together with a vulcanizing agent, for example, sulfur or sulfur with an accelerator may be employed. These indurating agents may be used separately or in combination and they are normally used in a proportion 95 not exceeding the bituminous material 100.

of the composition. In fact, it is preferable to use the indurating agents in a proportion between 10 and 100 parts of indurating agent per 100 parts of bituminous material.

- 5 For softening agents, I use, in general, that class of compounds ordinarily utilized for the purpose in rubber compounds, namely, petroleum, mineral oil, vegetable oil, rosin oil, etc. The proportion of softening agent used 10 is generally from 3 to 15 parts per 100 parts of bituminous material.

Fillers are added to the composition for the purpose of toughening the calender coat and reducing the cost. Finely divided solid 15 materials which are stable at the temperature of operation, such as whiting, lithopone, lime flour, litharge, iron oxide, carbon black, etc., are suitable for this use. However, finely divided fibrous materials, for example, asbestos, cotton linters, wood pulp and the like, 20 may be used, the filler being used in a proportion between 15 to 150 parts per 100 parts of bituminous material.

An oil varnish or an asphalt varnish, or a 25 varnish containing both drying oil and asphalt, may be used as a varnish coat. It is particularly advantageous to use an asphalt which softens at the baking temperature. In some cases one coat of drying oil varnish and a top coat of asphalt varnish may be used. However, the present invention is not limited to a product having a varnish coat, and it has been found that a superior product may be produced merely by calendering a bituminous 35 composition such as has been described, on to a suitable backing, and finishing by baking at a vulcanizing temperature.

The backing or base fabric may be any suitable material having the necessary strength 40 and flexibility; for instance, felt, cloth or paper.

The following is one example of the method of manufacturing artificial leather according to the present invention:

45 Two fabrics are combined with an adhesive rubber cement and upon the surface of this double fabric the following composition is calendered to a suitable thickness:

| Bituminous composition No. 1 |                      |          |
|------------------------------|----------------------|----------|
| Bituminous material          | Stearin pitch        | Parts 45 |
| Indurating agent             | Blown petroleum flux | 5        |
| Softening agent              | Reclaimed rubber     | 30       |
| Filler                       | Sulfur               | 0.5      |
|                              | Mineral oil          | 0.5      |
|                              | Whiting              | 10       |
|                              | Litharge             | 5        |
|                              | Lime flour           | 4        |
|                              |                      | 100.0    |

At this point the goods are embossed, a 50 grain suitable, for example, for automobile top material being used and a coat of asphalt-drying oil varnish applied, the material being then festooned in a vulcanizing chamber. The vulcanizing chamber is heated to the proper temperature which, in this case, is 60 about 123° C. and is maintained at this tem-

perature for 2½ hours. This heating operation not only vulcanizes the reclaimed rubber in the compound and hardens the bituminous material slightly, but also properly dries the finish coat of asphalt-drying oil varnish. The 70 particular asphalt varnish used has a larger proportion of asphalt than drying oil. It may sometimes be advisable to apply a base coat of black, drying oil varnish to the calendered embossed material before applying the 75 final coat of asphalt varnish. In this case, it is desirable to dry the first coat of varnish before the second is applied. This is accomplished by festooning the goods after applying the first coat of varnish and heating at 80 a temperature and for a length of time sufficient to dry the varnish properly.

The following are examples of variations of the bituminous coating composition which may be used in the above process according 85 to the invention and which fall within the limits which I have already described:

| Bituminous composition No. 2 |                      |          |
|------------------------------|----------------------|----------|
| Bituminous material          | Stearin pitch        | Parts 40 |
| Indurating agent             | Blown petroleum flux | 10       |
| Softening agent              | Smoked sheets        | 10       |
| Filler                       | Sulfur               | 0.4      |
|                              | Mineral oil          | 4        |
|                              | Whiting              | 30       |
|                              | Lime flour           | 2        |
|                              | Litharge             | 3.6      |
|                              |                      | 100.0 95 |

| Bituminous composition No. 3 |                   |          |
|------------------------------|-------------------|----------|
| Bituminous material          | Stearin pitch     | Parts 25 |
| Indurating agent             | Asphalt           | 25       |
| Filler                       | Hard brown factis | 15       |
|                              | Soft brown factis | 7.5      |
|                              | Whiting           | 27.5 100 |
|                              |                   | 100.0    |

A very desirable coating has been prepared by mixing together from 10 to 100 parts of the indurating agent, from 3 to 15 parts of the softening agent and from 15 to 150 parts of the filler to each 100 parts of the bituminous material, the bituminous material ranging from 30 to 80 per cent of the whole composition.

As compared with prior art products intended for similar purposes the coated fabric of the present invention has the advantage of low cost and long life especially under usage involving exposure to severe conditions of heat, cold, and direct sunlight. In addition, the bituminous calender coat as described has an advantage over known compositions for coating artificial leather, in that this calender coat provides a greatly improved support for any of the varnishes commonly used for finishing.

#### Claims:

1. A flexible fabric having a calender coat containing an indurating agent, a larger proportion of bituminous material than indurating agent, a softening agent and a filler and a varnish coating thereover.
2. The method of producing a coated fabric which includes the steps of mixing together an indurating agent, a larger amount

of bituminous material than indurating agent, a softening agent and a filler, coating a fabric backing with said mixture, festooning the coated fabric, and heating the said 5 coated fabric to a temperature of above 100° C. but below the decomposition point of the said mixture.

3. The method of producing a coated fabric which includes the steps of mixing together an indurating agent, a larger amount 10 of bituminous material than indurating agent, and a softening agent, coating a fabric backing with said mixture, festooning the coated fabric, and heating the said coated 15 fabric to a temperature of above 100° C. but below the decomposition point of the said mixture.

4. The method of producing a coated fabric which includes the steps of mixing together 100 parts bituminous material, 10 to 20 100 parts indurating agent, 3 to 15 parts softening agent and 15 to 150 parts filler, applying said mixture to a fabric, festooning the coated fabric, and subjecting the coated fabric 25 to a temperature sufficient to bake but not decompose said mixture.

5. The method of producing a coated fabric which includes the steps of forming a mixture of an indurating agent, a larger 30 amount of bituminous material than indurating agent, a softening agent and a filler, applying said mixture to a fabric, festooning the coated fabric, and heating said coated fabric to a temperature of above 100° C., but 35 below the decomposition point of the said mixture, for a period of 2½ hours.

In testimony whereof, I affix my signature.  
ARTHUR N. PARRETT.